# EUROPEAN PATENT SPECIFICATION

(11) **EP 0 652 935 B1**
(45) Date of publication and mention of the grant of the patent: **17.09.1997**
(21) Application number: 93915938.0
(22) Date of filing: 16.07.1993
(51) Int. Cl.: C11D 3/37, C11D 17/00, C08G 61/04, C08F 216/00

(54) **DETERGENT COMPOSITION**
WASCHMITTELZUSAMMENSETZUNG
COMPOSITION DETERGENTE

(30) Priority: 29.07.1992 EP 92306897
(43) Date of publication of application: 17.05.1995
(73) Proprietor: UNILEVER PLC, London EC4P 4BQ (GB); UNILEVER N.V., 3013 AL Rotterdam (NL)
(72) Inventor: KHOSHDEL, Ezat Unilever Res. Port Sunlight, GB-Wirral Merseyside L 63 3JW (GB); VAN DE PAS, Johannes Cornelis Unlilever Research, NL-3133 AT Vlaardingen (NL)
(74) Representative: Kan, Jacob Hendrik, Dr.
(86) International application number: EP9301882
(87) International publication number: WO9403575

(56) References cited:
- EP-A- 0 346 995
- EP-A- 0 415 698
- FR-A- 2 179 245
- FR-A- 2 179 246
- GB-A- 1 448 062
- DATABASE WPI Week 9010, Derwent Publications Ltd., London, GB; AN 90-071303
- DATABASE WPI Week 8901, Derwent Publications Ltd., London, GB; AN 89-004532
- DATABASE WPI Week 9104, Derwent Publications Ltd., London, GB; AN 91-025298

## Description

The present invention relates to deflocculating polymers and liquid detergent compositions comprising such polymers, in particular to liquid detergent compositions that comprise a dispersion of lamellar droplets in an aqueous continuous phase.

### Background & Prior art

Several types of deflocculating polymers are described in the art. EP 346 995 describes deflocculating polymers having a hydrophilic backbone and one or more hydrophobic side-chains, WO 91/06622 describes deflocculating polymers being a block copolymer consisting of alternating hydrophobic and hydrophilic groups, WO 91/06623 describes deflocculating polymers consisting of nonionic monomers and ionic monomers and GB 2 237 813 describes deflocculating polymers consisting of a hydrophobic backbone and one or more hydrophilic side-chains.

Deflocculating polymers have been used in liquid detergents, in particular in liquid detergent compositions that comprise a dispersion of lamellar droplets in an aqueous continuous phase, as for example described in EP 346 995, WO/91/06622, WO/91/06623 and GB 2 237 813. Other applications for deflocculating polymers in general purpose cleaners, liquid abrasive cleaners, liquid bleach compositions are disclosed in WO/91/09108, in fabric softening compositions in EP 415698 and the use in granular detergent compositions is disclosed in WO/91/09932.

WO/91/09109 discloses liquid detergent compositions comprising deflocculating polymers that are biodegradable.

As a consequence of consumers' and manufacturers' awareness for environmental issues, a trend can be seen to more development and more appreciation of "green" products, i.e. products with ingredients that are biodegraded quicker and easier, i.e. to search for ingredients that will result in an improved biodegradability of products.

Surprisingly, applicants have found a way to improve the biodegradability of deflocculating polymers.

These improved polymers do not suffer from loss of the beneficial deflocculating effects in liquid or granular detergent compositions. The improvement can be established by inclusion of a particular group in the hydrophilic backbone of the polymer, resulting in the polymers becoming better biodegradable.

### Definition of the invention

The matter for which protection is sought is defined in claims 1 to 8.

### Deflocculating polymer with hydrophilic backbone and one or more hydrophobic side-chains

Generally the hydrophilic backbone of the polymer is predominantly linear; the main chain or the backbone constitutes at least 50%, preferably more than 75%, most preferred more than 90% by weight of the polymer. Monomer units suitable for incorporation in the hydrophilic backbone are for example unsaturated C₁₋₆ acids, ethers, alcohols, aldehydes or esters, sugar units, alkoxy units, maleic anhydride and saturated polyalcohols such as glycerol. Examples of suitable monomer units are acrylic acid, alpha hydroxy acrylic acid, alpha hydroxy methyl acrylic acid, methacrylic acid, maleic acid, vinyl acetic acid, itaconic acid, polyethoxy groups preferably comprising from 4 to 50 ethylene oxide groups, polyglycerol, condensation polymers of polyglycerol and citric acid anhydride and condensation polymers of alpha-hydroxy acids or polyacetals.

Each of the above monomers can be present in the hydrophilic backbone in random order, in block arrangement or in mixtures thereof.

The hydrophilic backbone made from the backbone constituents in the absence of hydrophobic side-groups is relatively water-soluble at ambient temperature and a pH of between 6.5 and 14.0. Preferably the solubility is more than 1 g/l, more preferred more than 5 g/l most preferred more than 10 g/l.

Preferably the hydrophobic side chains are part of a monomer unit which is incorporated in the polymer by copolymerising hydrophobic monomers and the hydrophilic monomers making up the backbone of the polymer. The hydrophobic side chains for this use preferably include those which when isolated from their linkage are relatively water insoluble, i.e. preferably less than 1 g/l, more preferred less than 0.5 g/l, most preferred less than 0.1 g/l of the hydrophobic monomers, will dissolve in water at ambient temperature and a pH of 3.0 to 12.5.

Examples of relatively hydrophobic groups are butylene oxide and/or propylene oxide and/or alkyl or alkenyl chains. The hydrophobic groups may be connected to the hydrophilic backbone directly or via relatively hydrophilic linkages for example a polyethoxy linkage.

### Deflocculating polymer being a block copolymer having alternating hydrophobic and hydrophilic groups

These polymers have one of the following general structures: wherein A represents a hydrophobic group, B a hydrophilic group and z is an integer which is preferably zero.

The hydrophilic groups of the polymer are preferably composed of hydrophilic monomer units, which can be selected from a variety of units available for the preparation of polymers. Suitable hydrophilic monomer units are for instance described in the paragraph on deflocculating polymer with hydrophilic backbone and one or more hydrophobic side-chains. Particularly preferred hydrophilic groups are polyethoxy groups preferably comprising from 4 to 50 ethylene oxide groups, polyglycerol, condensation polymers of polyglycerol and citric acid anhydride and condensation polymers of alpha-hydroxy acids or polyacetals.

The hydrophobic groups of the polymer are preferably selected from saturated and unsaturated alkyl chains, e.g. having from 5 to 24 carbon atoms, preferably from 6 to 18, most preferred from 8 to 16 carbon atoms, and are optionally bonded to the adjacent hydrophilic groups via an alkoxylene or polyoxyalkylene linkage, for example a polypropoxy or butyloxy linkage having from 1 to 50 alkoxylene groups. Other suitable hydrophobic groups are polyoxyalkylene groups comprising from 4 to 50 propylene oxide and/or butylene oxide groups.

The hydrophilic groups may be linked to the hydrophobic groups by any possible chemical link, although the following types of linkages are preferred: -C-O-, -CO-O- or -O-.

### Deflocculating polymer with ionic and nonionic groups

The ionic-nonionic deflocculating polymer comprises a monomer A which is independently selected from the group of monomer units which are nonionic under the conditions in the liquid detergent product and a monomer B which is ionic under the conditions of the product.

Embraced in the definition of nonionic monomer A units for use in compositions of the invention are monomers which are nonionic of character under most circumstances and monomer units which are anionic or cationic of character, but which are at the conditions such as pH of the product neutralised such that they have an appreciable nonionic character. Preferably the pH of the product differs at least one unit, more preferred at least two units with the pKₐ value corresponding to the neutralisation of the monomer unit in the polymer.

Suitable monomer units which are nonionic per se are for example ethylenically unsaturated amides such as acrylamide, methacrylamide and fumaride and their N-substitued derivatives such as N-(dimethyl amino ethyl)acrylamide, vinyl alcohol, vinyl acetate, vinyl heterocyclic amides such as vinyl pyrrolidone, acrolein, allyl alcohol, hydroxy ethyl (meth) acrylate, hydroxy propyl (meth)acrylate, sugar units such as saccharides and glucosides, glycerol or other polyalcohols.

Suitable monomer units which are anionic at certain conditions, but which have an appreciable nonionic character at relatively low pH values of the product are for example: ethylenically unsaturated carboxylic acids, dicarboxylic acids such as acrylic acid, maleic acid, methacrylic acid, itaconic acid, fumaric acid, crotonic acid, aconitic acid and citraconic acid.

Suitable monomer units which are cationic under certain conditions, but which have an appreciable nonionic character at relatively high pH values are for example: amino alkyl esters of unsaturated carboxylic acids such as 2-amino ethyl (metha)crylate, dimethyl amino ethyl (meth)acrylate, diethyl amino ethyl (meth)acrylate, dimethyl amino methyl (meth) acrylate, diethyl amino ethyl (meth)acrylate, vinyl or alkyl amines such as vinyl pyridine, vinyl morpholine or allylamine.

Also mixtures of nonionic monomers may be used.

The ionic monomer B may be ionic under most circumstances, but also possible is the use of monomer units which only become ionised under the pH conditions of the product. If such ionisable monomer units are used, then preferably the pH of the product should differ at least one unit, more preferred at least two units with the pKₐ corresponding to the ionisation of the monomer in the polymer.

Examples of generally ionised monomer units are N(trimethylammoniumethyl) acrylamide chloride or sulphate, N(trimethyl ammonium propyl) acrylamide chloride or sulphate, 2-suphato ethyl (meth)acrylate and its ammonium, alkali metal or alkali earth metal salts, or can be obtained by conversion reactions of monomers A such as the cationisation of sugar units with 2,3 epoxypropyl trimethyl ammonium chloride, other ethylenically unsaturated quaternary ammonium compounds such as vinyl benzyl trimethyl ammonium chloride, the quaternary ammonium salts of di methyl/ethyl amino methyl/ethyl (meth)acrylate, vinyl aryl sulphonates such as vinyl benzyl sulphonate, sodium vinyl sulphonate, sodium alkyl sulphonate, beta-styrene phosphonic acid, sodium-p styrene sulphonate and vinyl phosphonic acid. Examples of monomer units which have an appreciable ionised character at relativly high pH values are ethylenically unsaturated carboxylic acids, dicarboxylic acids such as acrylic acid, maleic acid, methacrylic acid, itaconic acid, fumaric acid, crotonic acid, aconitic acid and citralinic acid.

Suitable monomer units which which have an appreciable ionised character at relatively low pH values are for example: amino alkyl esters of unsaturated carboxylic acids such as 2-amino ethyl (metha)crylate, dimethyl amino ethyl (meth)acrylate, diethyl amino ethyl (meth)acrylate, dimethyl amino methyl (meth) acrylate, diethyl amino ethyl (meth)acrylate, vinyl or alkyl amines such as vinyl pyridine, vinyl morpholine or allylamine.

Also mixtures of monomer units may be used.

Preferably the monomers for use in ionic-nonionic polymers are sufficiently hydrophilic to form at least a 1 % by weight solution when dissolved in water of ambient temperature and of the pH of the final product.

Preferably ionic-nonionic polymers contain at least two different monomers. The first of these monomers is preferably of nonionic character as defined hereinabove, the second monomer is preferably ionic under most circumstances as defined hereinabove. Most preferably the ionic monomer is a cationic monomer. Preferably the amount of ionic monomers in the polymer is from 0.1 to 50 % by weight of the polymer, more preferred from 1 to 25%, most preferred from 4 to 15%.

### Summary of the invention

A first group of preferred deflocculating polymers according to the present invention, having hydrophilic backbone and one or more hydrophobic side-chains, has the formula (I): wherein:
the monomer units may be in random order;
z is 1;
k is at least 1;
y preferably being from 0 up to the value of x;
n is at least 1 (and can be determined by the molecular weight);
the ratio of (k + x + y) : z is from 4 : 1 to 1,000 : 1, preferably from 6 : 1 to 250 : 1;
the ratio of k : (x + y + z) is from 1:99 to 30:70, preferably from 2:98 to 20:80, more preferably from 5:95 to 10:90;

R¹ represents -CO-O-, -O-, -O-CO-, -CH₂-, -CO-NH- or is absent;
R² represents from 1 to 50 independently selected alkyleneoxy groups (preferably ethylene oxide or propylene oxide groups), or is absent, provided that when R³ is absent and R⁴ represents hydrogen or contains no more than 4 carbon atoms, then R² contains at least 1 alkyleneoxy group, preferably more than 3, more preferably more than 5 alkyleneoxy groups, the alkyleneoxy groups preferably having at least 3 carbon atoms;
R³ represents a phenylene linkage, or is absent;
R⁴ represents hydrogen or a C₁₋₂₄ alkyl or C₂₋₂₄ alkenyl group, with the provision that when R² is absent, then R⁴ is not hydrogen and when also R³ is absent, then R⁴ contains at least 2, preferably at least 3, more preferably at least 4, most preferably at least 5 carbon atoms. More preferably R⁴ represents hydrogen or a C₁₋₂₄ alkyl or C₂₋₂₄ alkenylk group, with the provisos that:
   a) when R¹ represents -O-CO-, R² and R³ must be absent and R4 must contain at least 5 carbon atoms;
   b) when R² is absent, R⁴ is not hydrogen and when R³ is absent, then R⁴ must contain at least 5 carbon atoms.
R⁵ represents hydrogen or a group of formula -COOA⁴;
R⁶ represents hydrogen or C₁₋₄ alkyl; and

A¹, A², A³ and A⁴ are independently selected from hydrogen, alkali metals, alkaline earth metals, ammonium and amine bases and C₁₋₄, or (C₂H₄O)ₜH wherein t is from 1-50, and wherein the monomer units may be in random order.

Each B¹ is independently selected from -CH₂OH, -OH or -H;

For each monomer unit R¹-R⁶, A¹-A⁴ and B¹ may independently be selected from the groups mentioned above.

A second group of preferred deflocculating polymers of the present invention, having hydrophilic backbone and one or more hydrophobic side-chains, is of the formula (II): wherein: Q² is a molecular entity of formula (IIa): wherein:
the monomer units may be in random order;
z and v are 1;
n is at least 1 (and can be determined from the molecular weight);
k is at least 1;
at least 1 of the monomer units p, q or r is present;
the ratio of (k + x + y + p + q + r) : z is from 4 : 1 to 1,000 : 1, preferably from 6 : 1 to 250 : 1;
the ratio of k : (x + y + p + q + r + z) is from 1:99 to 30:70, preferably from 2:98 to 20:80, more preferably from 5:95 to 10:90;
R¹-R⁶, A¹-A⁴ and B¹ are as defined as for formula I.
R⁷ and R⁸ represent -CH₃ or -H;
R⁹ and R¹⁰ represent substituent groups such as amino, amine, amide, sulphonate, sulphate, phosphonate, phosphate, hydroxy, carboxyl and oxide groups, preferably they are selected from -SO₃Na, -CO-O-C₂H₄-OSO₃Na, -CO-O-NH-C(CH₃)₂-SO₃Na, -CO-NH₂, -O-CO-CH₃, -OH;

For each monomer unit R¹-R¹², A¹-A⁴ and B¹ may independently be selected from the groups mentioned above.

Q¹ is a multifunctional monomer, allowing the branching of the polymer, wherein the monomers of the polymer may be connected to Q¹ in any direction, in any order, therewith possibly resulting in a branched polymer. Preferably Q¹ is trimethyl propane triacrylate (TMPTA), methylene bisacrylamide or divinyl glycol.

A third group of preferred deflocculating polymers of the present invention, having hydrophilic backbone and one or more hydrophobic side-chains, and being especially suitable for fabric softening compositions comprising an aqueous base and one or more fabric-softening materials, is of the formula (III): wherein Q³ is derived from a monomeric unit IIIa comprising: Q⁴ is derived from the molecular entity IIIb: and Q⁵ is derived from a monomeric unit IIIc: wherein:
n is at least 1;
k is at least 1;
w is 0 to 4;
the ratio of (a + b + c + k) : d is from 5 : 1 to 500 : 1, in which the monomer units may be in random order, a, b, c, d, e, f, g, h may be integer or zero;
the ratio of k : (a + b + c + d) is from 1:99 to 30:70, preferably from 2:98 to 20:80, more preferably from 5:95 to 10:90;

R¹-R⁶ are defined as in formula I;
R¹¹ and R^{11*} are independently selected from hydrogen or C₁-C₄ alkyl;
R¹² is independently selected from C₅ to C₂₄ alkyl or alkenyl, aryl cycloalkyl, hydroxyalkyl or alkoxyalkyl; and
B¹, B², B³, B⁴ are organic or inorganic anions; the anions represented by B¹, B², B³, B⁴ are exemplified by the halide ions, sulphate, sulphonate, phosphate, hydroxide, borate, cyanide, carbonate, bicarbonate, thiocyanate, sulphide, cyanate, acetate and the other common inorganic and organic ions. Preferred anions are chloride and methosulphate.

A fourth group of preferred deflocculating polymers of the present invention, having hydrophilic backbone and one or more hydrophobic side-chains and being especially suitable for fabric softening compositions comprising an aqueous base and one or more fabric-softening materials, is of the formula (IV): wherein:
z is 1;
n is at least 1;
k is at least 1;
the ratio of (j + k) : z is from 5 : 1 to 500 : 1;
the ratio of k : (j + z) is from 1 : 99 to 30 : 70, preferably from 2 : 98 to 20 : 80, more preferably from 5 : 95 to 10 : 90; in which the monomer units may be in random order;

R¹-R⁶ are defined as in formula I;
R¹³ represents -CH₂-, -C₂H₄-, -C₃H₆ or is absent;
R¹⁴ represents from 1 to 50 independently selected alkyleneoxy groups, preferably ethylene oxide groups, or is absent.
R¹⁵ represents -H or -OH.

A fifth group of preferred deflocculating polymers of the present invention, having nonionic monomers and ionic monomers, is of the formula (V): wherein:
the monomer units may be in random order;
z is 1;
k is at least 1;
n is at least 1 (and can be determined from the molecular weight);
the ratio of (k + x) : z is from 1 : 1 to 2,000 : 1, preferably from 4 : 1 to 1,000 : 1 more preferably from 6 : 1 to 250 : 1;
the ratio of k : (x + z) is from 1:99 to 30:70, preferably from 2:98 to 20:80, more preferably from 5:95 to 10:90;

- R¹: represents -C₃H₆-N⁺-(CH₃)₃(Cl⁻⁾, -C₂H₄-OSO₃⁻⁽Na⁺), -SO₃⁻⁽Na⁺), -C₂H₄ N⁺(CH₃)₃ Cl^{-,} -C₂H₄ N⁺ (C₂H₆)₂ Cl⁻, -CH₂ N⁺ (CH₃)₃ Cl^{-,} -CH₂ N⁺ (C₂H₆)₂ Cl⁻ or benzyl-SO₃⁻ (Na⁺);
- R²: represents -CO-O-, -O-, -O-CO-, -CH₂-, -CO-NH-, or is absent;
- R³ and R⁴: represent hydrogen or C₁₋₄ alkyl;
- R^{a}: is CH₂, C₂H₄, C₃H₆ or is absent;
- R^{b}: represents form 1 to 50 independently selected alkylene oxide groups, preferably ethylene oxide groups or is absent;
- R^{c}: represents -OH or -H;
and wherein if R², R^{a} and R^{b} are absent, then R^{c} is not -H.

A sixth group of preferred deflocculating polymers of the present invention, being a block copolymer having alternating hydrophobic and hydrophilic groups is represented by the formulae (VI): wherein:
the monomer units may be in random order;
x is from 4 to 1,000, preferably from 6 to 250; k is at least 1;
the ratio of k : x is from 1:99 to 30:70, preferably from 2:98 to 20:80, more preferably from 5:95 to 10:90;

R¹ represents a C₂₋₂₄ alk(en)yl group, preferably C₃₋₂₄ alk(en)yl, more preferably C₅₋₂₄ alk(en)yl group, most preferably a C₆₋₂₄ alk(en)yl group, and/or from 4 to 50 propylene oxide or butylene oxide;
R² represents -CO-;
R³ represents -CO-O- or -O-.

The general formulae I-VI are to be construed as including those mixed copolymer forms wherein, within a particular polymer molcule where n is 2 or greater, R¹-R¹⁵ differ beetween individual monomer units therein.

### Molecular weight

Polymers for use in compositions may have a molecular weight between 500 and 1,000,000. The molecular weight is measured by GPC using polyethyleneglycol standards. For the purposes of this definition, the molecular weight of the standards are measured by the absolute intrinsic viscosity method described by Noda, Tsoge and Nagasawa in Journal of Physical Chemistry, Volume 74, (1970), page 710-719. Polymers according to the invention, preferably have molecular weights of from 750-100,000, more preferably of from 1,000 to 30,000, most preferably of from 2,000 to 10,000.

### Ketone group incorporation in the polymer

The polymers for use in detergent compositions of the invention may be prepared by using conventional polymerization procedures, such as radical polymerization, cationic-anionic polymerization or a combination thereof.

The ketone-group can be incorporated in the deflocculating polymer as described in our co-pending application GB 9207795.7 filed on 9 April 1992. The ketone groups can for example be derived from a compound of the formula (X): wherein each of R4 and R5, which may be the same or different, represents a group capable of stabilising a free radical.

Preferably, one of R4 and R5 represents an aryl or cyano group, and the other represents an aryl, alkyl or cyano group. Preferably at least one of R4 and R5 is a phenyl group, and the compound in which R4 and R5 both represent phenyl groups is especially preferred. This compound is 2,2-diphenyl-4-methylene-1,3-dioxolane.

On heating and in the presence of a free radical initiator, the ring of the monomer of the formula (X) opens. This product can be utilised to introduce a ketone functionality into the polymer by reaction with co-monomers.

### Biodegradability tests

Suitable tests for determining biodegradability are given in the OECD Guidelines. Other suitable tests involve the detection of released CO₂ upon decomposition of the polymer material, in these tests sometimes ¹⁴C labelled polymers may be used.

Preferably polymers for use in compositions of the invention satisfy one or more of the following tests:
(a) Modified SCAS test as described in OECD Guideline 302a. This test measures removal of test material by dissolved organic carbon analysis. It is believed that a 80 % removal is a reasonable indication of biodegradability or adsorption.
(b) Modified Sturm test as described in OECD Guideline 301b. This test measures CO₂ production from the test material under standard conditions, the polymer being enclosed in a sealed vessel inoculated with bacteria acclimatised to the test polymer in a sewage enrichment study. Values of 25 to 35% conversion to CO₂ in the modified Sturm test and similar tests have frequently been reported for polymers, but that can be attributed to the presence of monomers and low-molecular-weight oligomers. Values of 50% and above in this type of test are an indication of superior biodegradability. A 60 % conversion to CO₂ in the Sturm test is an indication of ready biodegradability.

Although it is preferred that polymers for use in composition of the invention satisfy both tests, applicants have found that polymers satisfying one biodegradability tests is suitable for use in the present invention.

### Product forms

Deflocculating polymers according to the invention can for example be used in liquid detergent composisitons, general purpose cleaners, liquid abrasive cleaners, liquid bleach compositions as disclosed in WO/91/09108 and also in granular detergent compositions as disclosed in WO/91/09932.

Deflocculating polymers can in particular be used in liquid detergent compositions that comprise a dispersion of lamellar droplets in an aqueous continuous phase.

Lamellar droplets are a particular class of surfactant structures which, inter alia, are already known from a variety of references, e.g. H.A.Barnes, 'Detergents', Ch.2. in K.Walters (Ed), 'Rheometry: Industrial Applications', J. Wiley & Sons, Letchworth 1980.

Such lamellar dispersions are used to endow properties such as consumer-preferred flow behaviour and/or turbid appearance. Many are also capable of suspending particulate solids such as detergency builders or abrasive particles. Examples of such structured liquids without suspended solids are given in US patent 4 244 840, whilst examples where solid particles are suspended are disclosed in EP-A-160 342; EP-A-38 101; EP-A-140 452 and also in the aforementioned US 4 244 840. Others are disclosed in EP-A-151 884, where the lamellar droplet are called 'spherulites'.

The presence of lamellar droplets in a liquid detergent product may be detected by means known to those skilled in the art, for example optical techniques, various rheometrical measurements, X-ray or neutron diffraction, and electron microscopy.

The droplets consist of an onion-like configuration of concentric bi-layers of surfactant molecules, between which is trapped water or electrolyte solution (aqueous phase). Systems in which such droplets are close-packed provide a very desirable combination of physical stability and solid-suspending properties with useful flow properties.

The viscosity and stability of the liquid product depend on the volume fraction of the liquid which is occupied by the droplets. Generally speaking, when the volume fraction is around 0.6, the droplets are just touching (space-filling).

This allows reasonable stability with an acceptable viscosity and endows useful solid-suspending properties.

Problems in formulating liquid detergent compositions of high lamellar phase volume are possible instability and/or high viscosity of the product, as described in our patent application EP 346 995. Compositions of the invention preferably have a viscosity of less than 2,500 mPas at 21 s-1, more preferred less than 1,500 mPas, most preferred less than 1,000 mPas, especially preferred between 100 and 750 mPas at 21 s-1.

Liquid compositions according to the invention are physically stable and have a relatively low viscosity, i.e. a corresponding composition minus the deflocculating polymer is less stable and/or has a higher viscosity. In the context of the present invention, physical stability for these systems can be defined in terms of the maximum separation compatible with most manufacturing and retail requirements. That is, the 'stable' compositions will yield no more than 10 %, preferably no more than 5 %, most preferred no more than 2% by volume phase separation as evidenced by appearance of 2 or more separate phases when stored at 25°C for 21 days from the time of preparation.

Preferably, liquid compositions of the invention comprising polymers according to formulae I, II, 2V and VI have a pH of between 6 and 14, more preferred from 6.5 to 13, especially preferred from 7 to 12. Preferably, liquid compositions of the invention comprising polymers according to formulae III and IV have a pH of less than 6.0, more preferred less than 5.0, especially from 1.5 to 4.5, most preferred from 2.0 to 4.0. Liquid compositions of the invention comprising polymers according to formulae I and II may also have low pH, i.e. more preferred less than 5.0, especially from 1.5 to 4.5, most preferred from 2.0 to 4.0.

The amount of the deflocculating polymer to be used is dependent on the product form in which it is used, as well as on the function in the product. In general the deflocculating polymer will be used at levels of from 0.01 to 5 % by weight of the composition, more preferably from 0.1 to 3.0, especially preferred from 0.25 to 2.0 %.

### Other ingredients

Compositions of the invention also comprise detergent active materials, preferably at a level of from 1 to 70% by weight of the composition, more preferred a level of 5 to 40 % by weight, most preferred from 10 to 35 % by weight.

In the case of blends of surfactants, the precise proportions of each component which will result in lamellar structures will depend on the type(s) and amount(s) of the electrolytes, as is the case with conventional structured liquids.

In the widest definition the detergent-active material in general, may comprise one or more surfactants, and may be selected from anionic, cationic, nonionic, zwitterionic and amphoteric species, and (provided mutually compatible) mixtures thereof. For example, they may be chosen from any of the classes, sub-classes and specific materials described in 'Surface Active Agents' Vol.I, by Schwartz & Perry, Interscience 1949 and 'Surface Active Agents' Vol.II by Schwartz, Perry & Berch (Interscience 1958), in the current edition of "McCutcheon's Emulsifiers & Detergents" published by the McCutcheon division of Manufacturing Confectioners Company or in 'Tensid-Taschenbuch', H.Stache, 2nd Edn., Carl Hanser Verlag, München & Wien, 1981.

Suitable nonionic surfactants include, in particular, the reaction products of compounds having a hydrophobic group and a reactive hydrogen atom, for example aliphatic alcohols, acids, amides or alkyl phenols with alkylene oxides, especially ethylene oxide, either alone or with propylene oxide. Specific nonionic detergent compounds are alkyl (C₆-C₁₈) primary or secondary linear or branched alcohols with ethylene oxide, and products made by condensation of ethylene oxide with the reaction products of propylene oxide and ethylenediamine. Other so-called nonionic detergent compounds include long chain tertiary amine oxides, long-chain tertiary phosphine oxides and dialkyl sulphoxides.

Preferably the level of nonionic surfactant materials is from 1 to 40 % by weight of the composition, more preferred from 2 to 20%.

Compositions of the present invention may contain synthetic anionic surfactant ingredients, which are preferably present in combination with the above mentioned nonionic materials. Suitable anionic surfactants are usually water-soluble alkali metal salts of organic sulphates and sulphonates having alkyl radicals containing from about 8 to about 22 carbon atoms, the term alkyl being used to include the alkyl portion of higher acyl radicals. Examples of suitable synthetic anionic detergent compounds are sodium and potassium alkyl sulphates, especially those obtained by sulphating higher (C₈-C₁₈) alcohols produced, for example, from tallow or coconut oil, sodium and potassium alkyl (C₉-C₂₀) benzene sulphonates, particularly sodium linear secondary alkyl (C₁₀-C₁₅) benzene sulphonates; sodium alkyl glycerol ether sulphates, especially those ethers of the higher alcohols derived from tallow or coconut oil and synthetic alcohols derived from petroleum; sodium coconut oil fatty monoglyceride sulphates and sulphonates; sodium and potassium salts of sulphuric acid esters of higher (C₈-C₁₈) fatty alcohol-alkylene oxide, particularly ethylene oxide, reaction products; the reaction products of fatty acids such as coconut fatty acids esterified with isethionic acid and neutralized with sodium hydroxide; sodium and potassium salts of fatty acid amides of methyl taurine; alkane monosulphonates such as those derived by reacting alpha-olefins (C₈-₂₀) with sodium bisulphite and those derived from reacting paraffins with SO₂ and Cl₂ and then hydrolyzing with a base to produce a random sulphonate; and olefin sulphonates, which term is used to describe the material made by reacting olefins, particularly C₁₀-C₂₀ alpha-olefins, with SO₃ and then neutralizing and hydrolyzing the reaction product. The preferred anionic detergent compounds are sodium (C₁₁-C₁₅) alkyl benzene sulphonates and sodium (C₁₆-C₁₈) alkyl sulphates.

Generally the level of the above mentioned non-soap anionic surfactant materials is from 1-40 % by weight of the composition, more preferred from 2 to 25 %. It is also possible, and sometimes preferred, to include an alkali metal soap of a mono- or di-carboxylic acid, especially a soap of an acid having from 12 to 18 carbon atoms, for example oleic acid, ricinoleic acid, alk(en)yl succinate for example dodecyl succinate, and fatty acids derived from castor oil, rapeseed oil, groundnut oil,coconut oil, palmkernel oil or mixtures thereof. The sodium or potassium soaps of these acids can be used. Preferably the level of soap in compositions of the invention is from 1-35% by weight of the composition, more preferred from 5-25%. Also possible is the use of salting out resistant active materials such as for example described in EP 328 177, especially the use of alkyl poly glycoside surfactants such as for example disclosed in EP 70 074. Also alkyl mono glucosides may be used.

The compositions optionally also contain electrolyte in an amount sufficient to bring about lamellar structuring of the detergent-active material. Preferably the compositions contain from 1% to 60%, especially from 10 to 45% of a salting-out electrolyte. Salting-out electrolyte has the meaning ascribed to in specification EP-A-79 646. Optionally, some salting-in electrolyte (as defined in the latter specification) may also be included.

In any event, it is preferred that compositions according to the present invention include detergency builder material, some or all of which may be electrolyte. In this context it should be noted that some detergent active materials such as for example soaps, also have builder properties.

Examples of phosphorous containing inorganic detergency builders include the water-soluble salts, especially alkali metalpyrophosphates, orthophosphates, polyphosphates and phosphonates. Specific examples of inorganic phosphate builders include sodium and potassium tripolyphosphates, phosphates and hexametaphosphates. Phosphonate sequestrant builders may also be used. Sometimes it is however preferred to minimise the amount of phosphate builders.

Examples of non-phosphorus-containing inorganic detergency builders, when present, include water-soluble alkali metal carbonates, bicarbonates, silicates and crystalline and amorphous aluminosilicates. Specific examples include sodium carbonate (with or without calcite seeds), potassium carbonate, sodium and potassium bicarbonates, silicates and zeolites.

In the context of inorganic builders, we prefer to include electrolytes which promote the solubility of other electrolytes, for example use of potassium salts to promote the solubility of sodium salts. Thereby, the amount of dissolved electrolyte can be increased considerably (crystal dissolution) as described in UK patent specification GB 1 302 543.

Examples of organic detergency builders, when present, include the alkaline metal, ammonium and substituted ammonium polyacetates, carboxylates, polycarboxylates, polyacetyl carboxylates and polyhydroxysulphonates. Specific examples include sodium, potassium, lithium, ammonium and substituted ammonium salts of ethylenediaminetetraacetic acid, nitrilotriacetic acid, oxydisuccinic acid, melitic acid, benzene polycarboxylic acids, CMOS, tartrate mono succinate, tartrate di succinate and citric acid. Citric acids or salts thereof are preferred builder materials for use in compositions of the invention.

In the context of organic builders, it is also desirable to incorporate polymers which are only partly dissolved, in the aqueous continuous phase as described in EP 301 882. This allows a viscosity reduction (due to the polymer which is dissolved) whilst incorporating a sufficiently high amount to achieve a secondary benefit, especially building, because the part which is not dissolved does not bring about the instability that would occur if substantially all were dissolved. Typical amounts are from 0.5 to 4.5% by weight.

It is further possible to include in the compositions of the present invention, alternatively, or in addition to the partly dissolved polymer, yet another polymer which is substantially totally soluble in the aqueous phase and has an electrolyte resistance of more than 5 grams sodium nitrilotriacetate in 100ml of a 5% by weight aqueous solution of the polymer, said second polymer also having a vapour pressure in 20% aqueous solution, equal to or less than the vapour pressure of a reference 2% by weight or greater aqueous solution of polyethylene glycol having an average molecular weight of 6000; said second polymer having a molecular weight of at least 1000. Use of such polymers is generally described in our EP 301,883. Typical levels are from 0.5 to 4.5% by weight.

Preferably the level of non-soap builder material is from 5-40 % by weight of the composition, more preferred from 5 to 25 % by weight of the composition.

### Optional ingredients

Apart from the ingredients already mentioned, a number of optional ingredients may also be present, for example lather boosters such as alkanolamides, particularly the monoethanolamides derived from palm kernel fatty acids and coconut fatty acids, lather depressants, oxygen-releasing bleaching agents such as sodium perborate and sodium percarbonate, peracid bleach precursors, chlorine-releasing bleaching agents such as trichloroisocyanuric acid, inorganic salts such as sodium sulphate, and, usually present in very minor amounts, fluorescent agents, perfumes, enzymes such as proteases, amylases and lipases (including Lipolase (Trade Mark) ex Novo), enzyme stabilizers, anti-redeposition agents, germicides and colorants.

Obviously in selecting the materials other than the polymer for use in compositions of the invention, also biodegradable materials are preferred for environmental reasons.

### Preparation of liquid detergent composition

Liquid compositions of the invention may be prepared by any conventional method for the preparation of liquid detergent compositions. A preferred method involves the dispersing of the electrolyte ingredient (if present) together with the minor ingredients except for the temperature sensitive ingredients -if any- in water of elevated temperature, followed by the addition of the builder material- if any-, the detergent active material (possibly as a premix) under stirring and thereafter cooling the mixture and adding any temperature sensitive minor ingredients such as enzymes perfumes etc. The deflocculating polymer may for example be added after the electrolyte ingredient or as the final ingredient. Preferably the deflocculating polymers are added prior to the formation of the lamellar structure.

In use the detergent compositions of the invention will be diluted with wash water to form a wash liquor for instance for use in a washing machine. The concentration of liquid detergent composition in the wash liquor is preferably from 0.1 to 10 %, more preferred from 0.1 to 3% by weight.

The invention will now be illustrated by way of the following non-limiting Examples.

### EXAMPLE I

| Synthesis of a deflocculating polymer: | |
|---|---|
| Ingredients | amount |
| Acrylic acid | 26.3 g (0.365 mole) |
| Lauryl methacrylate | 3.7 g (0.015 mole) |
| DMD ¹⁾ | 2.4 g (0.020 mole) |
| Sodium persulphate (4% aq) | 15 ml |
| Deionised water | 50 ml |
| Isopropanol | 25 ml |
| Sodium hydroxide | 13.9 g (0.320 mole) |

| | |
|---|---|
| ¹⁾ 2,2-diphenyl-4-methylene-1,3-dioxolane | |

### Procedure:

The water and isopropanol (IPA) was charged into a reaction vessel mounted in a heating bath thermostated at 100°C and degassed with oxygen free nitrogen. The DMD was dissolved in the acrylic acid-lauryl methacrylate by warming. The mixed monomer solution was then added dropwise over 3 hours to the stirred water/IPA solution. At the same time the persulphate initiator solution was fed in from another dropping funnel over a 4 hour period. After the addition was completed, the heating and stirring was continued for another 18 hours. This gave a sticky solid and an emulsion. 92 % of the theoretical amount of sodium hydroxide (in 30ml water) was added to achieve neutrality (pH 7). The IPA was removed by distillation using a rotary evaporator and the concentrate poured into acetone to precipitate the polymer and remove benzophenone. The polymer was separated, dissolved in water and precipitated again into acetone and the process repeated. Finally, the polymer was redissolved in water, filtered through glass fibre to remove the last traces of benzophenone then freeze-dried. Polymer yield 29.4g (94.5%). The polymer was characterised by 1H and 13C NMR, FT-IR and GPC. Molecular weights by aqueous GPC: Mn = 9,800 Mw = 32,200 D= 3.3.

### EXAMPLE 2

The following compositions were prepared by adding the citrate together with sufficient NaOH, to neutralise the active materials and to bring the pH of the final composition to 7, to water at a temperature of 30°C under stirring, followed by addition of the deflocculating polymer and a premix of the Synperonic and Dobs (in acid form).

| Basic composition 1: | |
|---|---|
| Ingredients | % (wt) |
| Na Dobs | 24.5 |
| Synperonic A7 | 9.9 |
| Na-citrate 2aq | 16.4 |
| Water | 49.2 |
| Deflocculation polymer | weights additional to basic formulation |

Polymer A is of the basic structure of formula I, wherein x = 24, k = 1, y = 0, R¹ is -CO-O-, R² and R³ are absent, R⁴ is -C₁₂H₂₅, R⁵ is -H, R⁶ is -CH₃, A¹ is Na and B¹ is -H. The molecular weight is 32,200.

The following results were obtained:

| No. | Basic Composition | Polymer | % | Stability | Viscosity m Pa.s at 21s⁻¹ |
|---|---|---|---|---|---|
| 1 | 1 | - | - | Unstable | 1750 - 2560^{*)} |
| 2 | 1 | A | 1.0 | Stable | 60 |

| | | | | | |
|---|---|---|---|---|---|
| ^{*)} Unreliable results due to rapid phase separation. | | | | | |

The polymer is also believe to have an acceptable biodegradability.

## Claims

1. Deflocculating polymer having a backbone wherein the polymer has a hydrophilic backbone and one or more hydrophobic side-chains, or is a block copolymer having alternating hydrophobic and hydrophilic groups, or has nonionic monomers and ionic monomers, characterised in that the deflocculating polymer comprises from 1 to 30 mole % of monomer units of the formula in the backbone.

2. A deflocculating polymer according to claim 1 characterised in that the polymer is of formula I: wherein:
the monomer units may be in random order;
z is 1;
k is at least 1;
n is at least 1 (and can be determined by the molecular weight);
the ratio of (k + x + y) : z is from 4 : 1 to 1,000 : 1; the ratio of k : (x + y + z) is from 1:99 to 30:70;
R¹ represents -CO-O-, -O-, -O-CO-, -CH₂-, -CO-NH- or is absent;
R² represents from 1 to 50 independently selected alkyleneoxy groups, or is absent, provided that when R³ is absent and R⁴ represents hydrogen or contains no more than 4 carbon atoms, then R² contains at least 1 alkyleneoxy group;
R³ represents a phenylene linkage, or is absent;
R⁴ represents hydrogen or a C₁₋₂₄ alkyl or C₂₋₂₄ alkenyl group, with the provision that when R² is absent, then R⁴ is not hydrogen and when also R³ is absent, then R⁴ contains at least 2 carbon atoms;
R⁵ represents hydrogen or a group of formula -COOA⁴;
R⁶ represents hydrogen or C₁₋₄ alkyl; and
A¹, A², A³ and A⁴ are independently selected from hydrogen, alkali metals, alkaline earth metals, ammonium and amine bases and C₁₋₄, or (C₂H₄O)ₜH wherein t is from 1 to 50, and wherein the monomer units may be in random order.
Each B¹ is independently selected from -CH₂OH, -OH or -H;
For each monomer unit R¹-R⁶, A¹-A⁴ and B¹ may independently be selected from the groups mentioned above;
formula (II): wherein: Q² is a molecular entity of formula (IIa): wherein:
the monomer units may be in random order;
z and v are 1;
n is at least 1 (and can be determined from the molecular weight);
k is at least 1;
at least 1 of the monomer units p, q or r is present;
the ratio of (k + x + y + p + q + r) : z is from 4 : 1 to 1,000 : 1;
the ratio of k : (x + y + p + q + r + z) is from 1:99 to 30:70;
R¹-R⁶, A¹-A⁴ and B¹ are as defined as for formula I.
R⁷ and R⁸ represent -CH₃ or -H;
R⁹ and R¹⁰ represent substituent groups such as amino, amine, amide, sulphonate, sulphate, phosphonate, phosphate, hydroxy, carboxyl and oxide groups, preferably they are selected from -SO₃Na, -CO-O-C₂H₄-OSO₃Na, -CO-O-NH-C(CH₃)₂-SO₃Na, -CO-NH₂, -O-CO-CH₃, -OH;
For each monomer unit R¹-R¹², A¹-A⁴ and B¹ may independently be selected from the groups mentioned above.
Q¹ is a multifunctional monomer, allowing the branching of the polymer, wherein the monomers of the polymer may be connected to Q¹ in any direction, in any order, therewith possibly resulting in a branched polymer; formula (III): wherein Q³ is derived from a monomeric unit IIIa comprising:
Q⁴ is derived from the molecular entity IIIb: and Q⁵ is derived from a monomeric unit IIIc:
wherein:
n is at least 1;
k is at least 1;
w is 0 to 4;
the ratio of (a + b + c + k) : d is from 5 : 1 to 500 : 1, in which the monomer units may be in random order, a, b, c, d, e, f, g, h may be integer or zero;
the ratio of k : (a + b + c + d) is from 1:99 to 30:70;
R¹-R⁶ are defined as in formula I;
R¹¹ and R^{11*} are independently selected from hydrogen or C₁-C₄ alkyl;
R¹² is independently selected from C₅ to C₂₄ alkyl or alkenyl, aryl cycloalkyl, hydroxyalkyl or alkoxyalkyl; and
B¹, B², B³, B⁴ are organic or inorganic anions; the anions represented by B¹, B², B³, B⁴ are exemplified by the halide ions, sulphate, sulphonate, phosphate, hydroxide, borate, cyanide, carbonate, bicarbonate, thiocyanate, sulphide, cyanate, acetate and the other common inorganic and organic ions;
formula (IV):
wherein:
z is 1;
n is at least 1;
k is at least 1;
the ratio of (j + k) : z is from 5 : 1 to 500 : 1;
the ratio of k : (j + z) is from 1 : 99 to 30 : 70; in which the monomer units may be in random order;
R¹-R⁶ are defined as in formula I;
R¹³ represents -CH₂-, -C₂H₄-, -C₃H₆ or is absent;
R¹⁴ represents from 1 to 50 independently selected alkyleneoxy groups, preferably ethylene oxide groups, or is absent.
R¹⁵ represents -H or -OH;
formula (V):
wherein:
the monomer units may be in random order;
z is 1;
k is at least 1;
n is at least 1 (and can be determined from the molecular weight);
the ratio of (k + x) : z is from 1 : 1 to 2,000 : 1; the ratio of k : (x + z) is from 1:99 to 30:70;
R¹ represents -C₃H₆-N⁺-(CH₃)₃(Cl⁻), -C₂H₄-OSO₃⁻⁽Na⁺), -SO₃⁻⁽Na⁺), -C₂H₄ N⁺(CH₃)₃ Cl^{-,} -C₂H₄ N⁺ (C₂H₆)₂ Cl⁻, -CH₂ N⁺ (CH₃)₃ Cl^{-,} -CH₂ (C₂H₆)₂ Cl⁻ or benzyl-SO₃⁻ (Na⁺);
R² represents -CO-O-, -O-, -O-CO-, -CH₂-, -CO-NH-, or is absent;
R³ and R⁴ represent hydrogen or C₁₋₄ alkyl;
R^{a} is CH₂, C₂H₄, C₃H₆ or is absent;
R^{b} represents form 1 to 50 independently selected alkylene oxide groups, preferably ethylene oxide groups or is absent;
R^{c} represents -OH or -H;
and wherein if R², R^{a} and R^{b} are absent, then R^{c} is not -H; or
formulae (VI): wherein:
the monomer units may be in random order;
x is from 4 to 1,000;
k is at least 1;
the ratio of k : x is from 1:99 to 30:70;
R¹ represents a C₂₋₂₄ alk(en)yl group and/or from 4 to 50 propylene oxide or butylene oxide;
R² represents -CO-;
R³ represents -CO-O- or -O-.

3. A liquid detergent composition comprising a dispersion of lamellar droplets of detergent active material in an aqueous continuous phase and further comprising a deflocculating polymer according to claim 1.

4. A liquid detergent composition according to claim 3 characterised in that the amount of deflocculating polymer is from 0.01 to 5% by weight of the composition.

5. A liquid detergent composition according to claim 3 characterised in that the deflocculating polymers satisfies at least one of biodegradability tests selected from the Modified SCAS test and the Modified Sturm test.

6. A liquid detergent composition according to claim 3 characterised in that the viscosity of the liquid is less than 2,500 mPas at 21 s⁻¹.

7. A liquid detergent composition according to claim 3 characterised in that the liquid comprises from 1-70% by weight of detergent active material.

8. A liquid detergent composition according to claim 3 characterised in that the liquid yields less than 10% by volume phase separation when stored at 25°C for 21 days from the day of preparation.

## Patentansprüche

1. Entflockendes Polymer mit einem Gerüst, bei dem das Polymer ein hydrophiles Gerüst und eine oder mehrere hydrophobe Seitenketten aufweist oder ein Blockcopolymer mit abwechselnden hydrophoben und hydrophilen Gruppen ist oder nichtionische Monomere und ionische Monomere aufweist, **dadurch gekennzeichnet**, daß das entflockende Polymer 1 bis 30 Mol-% Monomereinheiten der Formel im Gerüst enthält.

2. Entflockendes Polymer nach Anspruch 1, **dadurch gekennzeichnet**, daß das Polymer die Formel I: hat, worin die Monomereinheiten statistisch angeordnet sein können;
z 1 ist;
k mindestens 1 ist;
n mindestens 1 ist (und durch das Molekulargewicht bestimmt werden kann);
das Verhältnis von (k + x + y) : z 4:1 bis 1.000:1 ist;
das Verhältnis von k : (x + y + z) 1:99 bis 30:70 ist;
R¹ -CO-O-, -O-, -O-CO-, -CH₂-, -CO-NH- bedeutet oder nicht vorhanden ist;
R² 1 bis 50 unabhängig ausgewählte Alkylenoxygruppen bedeutet oder nicht vorhanden ist, mit dem Vorbehalt, daß dann, wenn R³ nicht vorhanden ist und R⁴ Wasserstoff bedeutet oder nicht mehr als 4 Kohlenstoffatome enthält, daß dann R² mindestens eine Alkylenoxygruppe enthält;
R³ eine Phenylen-Bindungsgruppe bedeutet oder nicht
R⁴ Wasserstoff oder eine C₁₋₂₄-Alkyl- oder C₂₋₂₄-Alkenylgruppe bedeutet, mit dem Vorbehalt, daß dann wenn R² nicht vorhanden ist, R⁴ nicht Wasserstoff ist und wenn auch R³ nicht vorhanden ist, R⁴ mindestens 2 Kohlenstoffatome enthält;
R⁵ Wasserstoff oder eine Gruppe der Formel -COOA⁴ bedeutet;
R⁶ Wasserstoff oder einen C₁₋₄-Alkylrest bedeutet und A¹, A², A³ und A⁴ unabhängig ausgewählt sind aus Wasserstoff, Alkalimetallen, Erdalkalimetallen, Ammonium- und Aminbasen und C₁₋₄-Resten oder (C₂H₄O)ₜH, worin t 1 bis 50 ist, wobei die Monomereinheiten in statistischer Anordnung sein können;
jeder Rest B¹ unabhängig ausgewählt ist aus -CH₂OH, -OH oder -H;
für jede Monomereinheit R¹-R⁶, A¹-A⁴ und B¹ unabhängig aus den oben erwähnten Gruppen ausgewählt werden können; die Formel (II): hat, worin Q² eine molekulare Einheit der Formel (IIa) : ist, worin die Monomereinheiten statistisch angeordnet sein können;
z und v 1 sind;
n mindestens 1 ist (und aus dem Molekulargewicht bestimmt werden kann);
k mindestens 1 ist;
in mindestens einer der Monomereinheiten p, q oder r vorhanden ist; das Verhältnis von (k + x + y + p + q + r) : z 4:1 bis 1.000:1 ist;
das Verhältnis von k : (x + y + p + q + r + z) 1:99 bis 30:70 ist;
R¹-R⁶, A¹-A⁴ und B¹ wie für Formel I definiert sind;
R⁷ und R⁸ -CH₃ oder -H bedeuten;
R⁹ und R¹⁰ Substituentengruppen bedeuten, wie Amino-, Amin-, Amid-, Sulfonat-, Sulfat-, Phosphonat-, Phosphat-, Hydroxyl-, Carboxyl- und Oxidgruppen, und bevorzugt ausgewählt sind aus -SO₃Na, -CO-O-C₂H₄-OSO₃Na, -CO-O-NH-C(CH₃)₂-SO₃Na, -CO-NH₂, -O-CO-CH₃, -OH;
für jede Monomereinheit R¹-R¹², A¹-A⁴ und B¹ unabhängig aus den oben erwähnten Gruppen ausgewählt werden können;
Q¹ ein multifunktionelles Monomer ist, das eine Verzweigung des Polymers zuläßt, wobei die Monomere des Polymers mit Q¹ in jeder Richtung, in jeder Anordnung verbunden sein können, wodurch möglicherweise ein verzweigtes Polymer entsteht;
die Formel (III): hat, worin Q³ von einer monomeren Einheit IIIa abgeleitet ist, die: umfaßt,
Q⁴ von der Moleküleinheit IIIb: abgeleitet ist und
Q⁵ von einer Monomereinheit IIIc: abgeleitet ist,
worin
n mindestens 1 ist;
k mindestens 1 ist;
w 0 bis 4 ist;
das Verhältnis von (a + b + c + k) : d 5:1 bis 500:1 ist, worin die Monomereinheiten statistisch angeordnet sein können, a, b, c, d, e, f, g, h ganze Zahlen oder 0 sein können;
das Verhältnis von k : (a + b + c + d) 1:99 bis 30:70 ist;
R¹-R⁶ wie in Formel I definiert sind;
R¹¹ und R^{11*} unabhängig ausgewählt sind aus Wasserstoff oder C₁-C₄-Alkylresten;
R¹² unabhängig ausgewählt ist aus C₅-C₂₄-Alkyl- oder Alkenyl-, Aryl-, Cycloalkyl-, Hydroxyalkyl- oder Alkoxyalkylresten und
B¹, B², B³, B⁴ organische oder anorganische Anionen sind; wobei Beispiele für die durch B¹, B², B³, B⁴ dargestellten Anionen Halogenidionen, Sulfat-, Sulfonat-, Phosphat-, Hydroxid-, Borat-, Cyanid-, Carbonat-, Bicarbonat-, Thiocyanat-, Sulfid-, Cyanat-, Acetat- und andere übliche anorganische und organische Ionen sind;
die Formel (IV): hat, worin
z 1 ist;
n mindestens 1 ist;
k mindestens 1 ist;
das Verhältnis von (j + k) : z 5:1 bis 500:1 ist;
das Verhältnis von k : (j + z) 1:99 bis 30:70 ist; worin die Monomereinheiten statistisch angeordnet sein können;
R¹-R⁶ wie für Formel I definiert ist;
R¹³ -CH₂-, -C₂H₄-, -C₃H₆ bedeutet oder nicht vorhanden ist;
R¹⁴ 1 bis 50 unabhängig ausgewählte Alkylenoxygruppen, bevorzugt Ethylenoxidgruppen bedeutet, oder nicht vorhanden ist;
R¹⁵ -H oder -OH bedeutet;
die Formel (V): hat, worin die Monomereinheiten statistisch angeordnet sein können;
z 1 ist;
k mindestens 1 ist;
n mindestens 1 ist (und aus dem Molekulargewicht bestimmt werden kann);
das Verhältnis von (k + x) : z 1:1 bis 2.000:1 ist;
das Verhältnis von k : (x + z) 1:99 bis 30:70 ist;
R¹ -C₃H₆-N⁺-(CH₃)₃(Cl⁻), -C₂H₄-OSO₃⁻(Na⁺), -SO₃⁻(Na⁺), -C₂H₄N⁺(CH₃)₃Cl⁻, -C₂H₄N⁺(C₂H₆)₂Cl⁻, -CH₂N⁺(CH₃)₃Cl⁻, -CH₂N⁺(C₂H₆)₂Cl⁻ oder Benzyl-SO₃⁻(Na⁺) bedeutet;
R² -CO-O-, -O-, -O-CO-, -CH₂-, -CO-NH- bedeutet oder nicht vorhanden ist;
R³ und R⁴ Wasserstoff oder C₁₋₄-Alkylreste bedeuten;
R^{a} CH₂, C₂H₄, C₃H₆ bedeutet oder nicht vorhanden ist;
R^{b} 1 bis 50 unabhängig ausgewählte Alkylenoxidgruppen, bevorzugt Ethylenoxidgruppen bedeutet oder nicht vorhanden ist;
R^{c} -OH oder -H bedeutet;
und worin, wenn R², R^{a} und R^{b} nicht vorhanden sind, R^{c} nicht -H ist oder
die Formel (VI): hat, worin die Monomereinheiten statistisch angeordnet sein können;
x 4 bis 1.000 ist;
k mindestens 1 ist;
das Verhältnis k:x 1:99 bis 30:70 ist;
R¹ eine C₂₋₂₄-Alk(en)ylgruppe und/oder 4 bis 50 Propylenoxid- oder Butylenoxid-Einheiten bedeutet;
R² -CO- ist;
R³ -CO-O- oder -O- ist.

3. Flüssig-Waschmittel-Zusammensetzung enthaltend eine Dispersion lamellarer Tröpfchen aus waschaktivem Material in einer wäßrigen kontinuierlichen Phase und weiter enthaltend ein entflockendes Polymer nach Anspruch 1.

4. Flüssig-Waschmittel-Zusammensetzung nach Anspruch 3, **dadurch gekennzeichnet**, daß die Menge an entflockendem Polymer 0,01 bis 5 Gew.-%, bezogen auf die Zusammensetzung, ist.

5. Flüssig-Waschmittel-Zusammensetzung nach Anspruch 3, **dadurch gekennzeichnet**, daß das entflockende Polymer mindestens einen Test zur biologischen Abbaubarkeit, ausgewählt aus dem modifizierten SCAS-Test und dem modifizierten Sturm-Test, erfüllt.

6. Flüssig-Waschmittel-Zusammensetzung nach Anspruch 3, **dadurch gekennzeichnet**, daß die Viskosität der Flüssigkeit kleiner als 2.500 mPas bei 21 s⁻¹ ist.

7. Flüssig-Waschmittel-Zusammensetzung nach Anspruch 3, **dadurch gekennzeichnet**, daß die Flüssigkeit 1 bis 70 Gew.-% waschaktives Material enthält.

8. Flüssig-Waschmittel-Zusammensetzung nach Anspruch 3, **dadurch gekennzeichnet**, daß die Flüssigkeit weniger als 10 Vol.-% Phasentrennung liefert, wenn sie bei 25°C 21 Tage vom Tag der Herstellung an aufbewahrt wird.

## Revendications

1. Polymère défloculant ayant un squelette, dans lequel le polymère a un squelette hydrophile et une ou plusieurs chaînes latérales hydrophobes, ou est un copolymère bloc ayant une alternance de groupes hydrophobes et hydrophiles, ou a des monomères non ioniques et des monomères ioniques, caractérisé en ce que le polymère défloculant comprend de 1 à 30 moles % d'unités monomères de la formule : dans le squelette.

2. Un polymère défloculant selon la revendication 1, caractérisé en ce que le polymère a la formule I : dans laquelle :
les unités monomères peuvent être dans un ordre aléatoire ;
z est 1
k est au moins 1
n est au moins 1 (et peut être déterminé par la masse moléculaire) ;
le rapport de (k + x + y) : Z va de 4 pour 1 à 1,000 pour 1 ;
le rapport k : (x + y + z) va de 1 pour 99 à 30 pour 70;
R¹ représente -CO-O-, -O-, -O-CO-, -CH₂-, -CO-NH- ou est absent ;
R² représente de 1 à 50 groupes alkylènoxy sélectionnés de façon indépendante, ou est absent, à condition que R³ soit absent et que R⁴ représente l'hydrogène ou ne contienne pas plus de 4 atomes de carbone, et dans ce cas R² contient au moins 1 groupe alkylènoxy;
R³ représente une liaison phénylène ou est absent ;
R⁴ représente de l'hydrogène ou un groupe alkyle en C₁₋₂₄ ou un groupe alkényle en C₂₋₂₄, à condition que lorsque R² est absent, alors R⁴ n'est pas de l'hydrogène, et à condition que lorsque R³ est également absent, alors R⁴ contient au moins 2 atomes de carbone;
R⁵ représente de l'hydrogène ou un groupe de formule -COOA⁴ ;
R⁶ représente de l'hydrogène ou un alkyle en C₁₋₄ ; et
A¹, A², A³ et A⁴ sont indépendamment sélectionnés à partir de l'hydrogène, des métaux alcalins, des métaux alcalino-terreux, des bases ammonium et amines, des C₁₋₄, ou (C₂H₄O)ₜH dans lequel t va de 1 à 50 et dans lesquels les unités monomères peuvent être dans un ordre aléatoire.
Chaque B¹ est indépendamment sélectionné à partir de -CH₂OH-, -OH ou -H ;
Pour chaque unité monomère, R¹-R⁶, A¹-A⁴ et B¹ peuvent être indépendamment sélectionnés à partir des groupes mentionnés ci dessus.
formule (II) : dans laquelle Q² est une entité moléculaire de formule (IIa) : dans laquelle :
les unités monomères peuvent être en ordre aléatoire ;
z et v sont 1 ;
n est au moins 1 (et peut être déterminé à partir de la masse moléculaire) ;
k est au moins 1 ;
au moins une des unités monomères p, q ou r est présente ;
le rapport de (k + x + y + p + q + r) : z va de 4 pour 1 à 1.000 pour 1;
le rapport de k : (x + y + p + q + r + z) va de 1 pour 99 à 30 pour 70 ;
R¹ - R⁶, A¹ - A⁴ et B¹ sont tels que définis dans la formule I.
R⁷ et R⁸ représentent -CH₃ ou -H ;
R⁹ et R¹⁰ représentent des groupes de substitution tels que des groupes aminos, amines, amides, sulphonates, sulfates, phosphonates, phosphates, hydroxy, carboxyles et oxydes ; ils sont de préférence sélectionnés à partir de -SO₃Na, -CO- O-C₂H₄-OS₃Na, -CO-O-NH-C(CH₃)₂-SO₃Na, -CO-NH₂, -O-CO-CH₃, -OH ;
Pour chaque unité monomère, R¹ - R¹², A¹ - A⁴ et B¹ peuvent être sélectionnés indépendant parmi les groupes mentionnés ci dessus.
Q¹ est un monomère multifonctionnel permettant la ramification du polymère, dans laquelle les monomères ou le polymère peuvent être reliés à Q¹ dans n'importe quelle direction, dans n'importe quel ordre, ce qui peut avoir pour résultat un polymère ramifié.
Formule (III) : dans laquelle Q³ est dérivé d'une unité monomère IIIa comprenant : Q⁴ est dérivé de l'entité moléculaire IIIb : et Q⁵ est dérivé de l'unité monomère IIIc : dans laquelle :
n est au moins 1 ;
k est au moins 1 ;
w va de 0 à 4 ;
le rapport de (a + b + c + k) : d va de 5 pour 1 à 500 pour 1 ;
dans laquelle les unités monomères peuvent être en ordre aléatoire, a, b, c, d, e, f, g, h peuvent être des nombres entiers ou zéro ;
le rapport de k : (a + b + c + d) va de 1 pour 99 à 30 pour 70 ;
R¹ - R⁶ sont définis tel que dans la formule I ;
R¹¹ et R^{11*} sont indépendamment sélectionnés à partir de l'hydrogène ou de l'alkyle en C₁ - C₄ ;
R¹² est indépendamment sélectionné parmi les alkyles en C₅ à C₂₄, les alkényles, les aryl cycloalkyles, les hydroxyalkyles ou les hydroxyalkyles ; et
B¹, B², B³ et B⁴ sont des anions organiques ou inorganiques ; des exemples des anions représentés par B¹, B², B³ et B⁴ sont les ions halides, le sulfate, le sulphonate, le phosphate, l'hydroxyde, le cyanide, le carbonate, le bicarbonate, le thiocyanate, le sulphide, le cyanate, l'acétate et les autres ions communs inorganiques et organiques.
Formule (IV) : dans laquelle :
z est 1 ;
n est au moins 1 ;
k est au moins 1
le rapport de (j + k) : z va de 5 pour 1 à 500 pour 1 ;
le rapport de k : (j + z) va de 1 pour 99 à 30 pour 70 ; dans laquelle les unités monomère peuvent être en ordre aléatoire ;
R¹⁻ R⁶ sont tels que définis dans la formule I ;
R¹³ représente -CH₂-, - C₂H₄-, -C₃H₆ ou est absent ;
R¹⁴ représente de 1 à 50 groupes alkylèneoxy sélectionnés de façon indépendante, de préférence des groupes d'oxyde d'éthylène, ou il est absent ;
R¹⁵ représente -H ou -OH.
Formule (V) : dans laquelle :
les unités monomères peuvent être en ordre aléatoire ;
z est 1
k est au moins 1 ;
n est au moins 1 (et peut être déterminé à partir de la masse moléculaire) ;
le rapport de (k + x) : z va de 1 pour 1 à 2.000 pour 1 ;
le rapport de k : (x + y) va de 1 pour 99 à 30 pour 70 ;
R¹ représente -C₃H₆ - N⁺ -(CH₃)₃(Cl⁻), -C₂H₄ - OSO₃⁻ (Na⁺), -SO₃⁻ (Na⁺), -C₂H₄N⁺ (CH₃)₃ Cl⁻, -C₂H₄N⁺ (C₂H₆)₂ Cl⁻, -CH₂ N⁺ (CH₃)₃ Cl⁻, -CH₂N⁺ (C₂H₆)₂ Cl⁻ ou benzyl- SO₃⁻ (Na⁺) ;
R² représente -CO-O-, -O-, -O-CO-, -CH₂-, -CO-NH-, ou est absent ;
R³ et R⁴ représentent de l'hydrogène ou un alkyle en C₁₋₄ ;
R^{a} est CH₂, C₂H₄, C₃H₆ ou est absent,
R^{b} représente de 1 à 50 de 1 à 50 groupes d'oxyde d'alkylène sélectionnés de façon indépendante, de préférence des groupes d'oxyde d'éthylène, ou est absent ;
R^{c} représente -OH ou -H ;
et dans laquelle si R², R^{a} et R^{b} sont absents alors R^{c} n'est pas -H ;
ou
Formule (VI) : dans laquelle :
les unités monomères peuvent être en ordre aléatoire ;
x va de 4 pour 1.000 ;
k est au moins 1 ;
le rapport de k sur x va de 1 pour 99 à 30 pour 70 ;
R¹ représente un groupe alk(én)yle en C₂₋₂₄ et/ou de 4 à 50 groupes d'oxyde de propylène ou d'oxyde de butylène;
R² représente -CO- ;
R³ représente -CO-O- ou -O-.

3. Une composition détergente liquide comprenant une dispersion de gouttelettes lamellaires de matériau détergent actif dans une phase aqueuse continue et comprenant en outre un polymère défloculant selon la revendication 1.

4. Une composition détergente liquide selon la revendication 3, caractérisée en ce que la quantité de polymère défloculant va de 0,01 à 5 % en masse de la composition.

5. Une composition détergente liquide selon la revendication 3, caractérisée en ce que le polymère défloculant satisfait à au moins un des essais de biodégradabilité choisi entre l'essai SCAS Modifié et l'essai Sturm Modifié.

6. Une composition détergente liquide selon la revendication 3, caractérisée en ce que la viscosité du liquide est au moins inférieure à 2.500 mPas à 21 s⁻¹.

7. Une composition détergente liquide selon la revendication 3, caractérisée en ce que le liquide comprend de 1 à 70 % en masse de matériau détergent actif.

8. Une composition détergente liquide selon la revendication 3, caractérisée en ce que le liquide produit moins de 10 % de séparation de phase lorsqu'il est stocké à 25°C pendant 21 jours à compter du jour de la préparation.
